

# UNITED STATES PATENT OFFICE.

CHILD HAROLD WILLS, OF DETROIT, MICHIGAN.

## ALLOY STEEL.

1,278,082.

Specification of Letters Patent.

Patented Sept. 3, 1918.

No Drawing.

Application filed June 9, 1917. Serial No. 173,719.

*To all whom it may concern:*

Be it known that I, CHILD HAROLD WILLS, a citizen of the United States, residing at Detroit, in the county of Wayne and State 5 of Michigan, have invented certain new and useful Improvements in Alloy Steels, of which the following is a specification.

This invention relates to alloy steels, and particularly to what may be termed commercial steels. The nature of my invention, its 10 objects and advantages will be best understood from a brief statement of what is comprehended by "commercial steels" and the properties and characteristics such steels 15 must have to bring them within this category.

Broadly speaking, there are four general factors or considerations affecting the commercial possibilities of all alloy steel: first, 20 the making of the steel itself; second, the manufacture of articles from the steel; third, the performance of the article produced, *i. e.*, the properties of the finished article; and fourth, the cost, which materially enters 25 into the first two named considerations. The second factor may be further classified into three general divisions; namely, the forming of the steel into the article, the heat treatment, and the machining or working. 30 A varying number of considerations enter into each general factor.

Thus, for example, in the making of the steel, it is desirable, on the score of expense and other grounds, that the melting be done 35 by the open hearth method. It is also essential that the alloys be capable of ladle addition, and that segregation, or the formation of pockets of the alloy, be prevented. Segregation frequently occurs, as for example, 40 in manganese steels. Again, the loss of alloys in remelting must be kept within reasonable limits, as must the amount of the alloy required, as determined for example, by the output available. In so far as casting 45 is concerned, the ingots should be smooth and should have good preliminary rolling or characteristics such as clean surfaces, with a minimum amount of chipping necessary. Finally, the cropping must be kept within 50 reasonable limits, and the scrap after final rolling into bar form should be small and capable of being handled without loss. Stated in other words in addition to the

other factors above set forth, the yield should be large.

If an alloy steel materially fails to meet these important requirements of the steel maker, it may at once be ruled out as a commercial steel, although it may be useful for such special purposes as warrant the high 60 cost of making.

As to the manufacture or forming of the alloy steel into the desired articles, the steel should be capable of being forged or drop hammered at a high temperature, because 65 the greater plasticity of the metal materially cuts down the forging operations. At the same time, however, the steel must be of such a character that no marked or undue crystallization or other detrimental structural change takes place at the high forging temperature. In this connection, the chief difficulty encountered in commercial alloy steels is that at high forging temperatures even under the point at which burning of 70 the metal takes place there occurs loss of certain properties or characteristics which no subsequent heat treatment can reclaim. Thus, for example, in the vanadium steels at present so largely used in the manufacture of automobile parts, at temperatures from the point of recalescence upward, the 75 size of the crystals increases with great rapidity and structural changes develop which are detrimental to elongation and reduction 80 of area even after the steel has subsequently been heat treated. The allowable forging temperature limits are thus quite restricted, and because of the difficulty of maintaining furnace temperatures uniform, as will 85 be readily understood by those skilled in the art, it frequently happens that the limits are exceeded, with crystallization and consequent weakness as the result. In addition 90 to the foregoing, the steel should have good welding characteristics, should be non-air hardening, and substantially free from the 95 formation of seams and pipes.

As to heat treatment, after forming or forging, using vanadium steel for purposes of illustration, it is customary to subject the steel to three heats, a normalizing heat, a quenching heat, and a drawing heat, to which may be added a fourth heat for case-hardening purposes, where such is required. The chief difficulties encountered in this

connection are losses which occur because, in the first place, commercial alloy steels are very sensitive to heat treatment, *i. e.*, the range of temperature within which they must be heat treated is very narrow, and in the second place, it is impossible to maintain furnace temperatures uniform. If the steel be treated at a temperature too low, it lacks the desired properties; if treated at a temperature too high, it will be crystallized, or even burned, *i. e.*, it will undergo certain structural changes which subsequent heat treatment will not rectify. Such steels will not measure up to the requirements of the service for which they are intended, as the beneficial effects of the alloys are lost. To meet these conditions, it is customary to provide complicated regulating equipment, involving a large item of expense, but even such equipment is not productive of uniformly satisfactory results, and the percentage of losses in manufacture and service, although reduced, is still quite large. It will be apparent that an ideal commercial steel would be one which, instead of being sensitive to heat treatment, would have a wide range of temperature, for reasons which will further appear.

Another factor entering into heat treating operations is that minimum crystallization should take place during carburizing.

As to the workability of commercial alloy steels, it is requisite that they can be readily machined and worked after heat treatment.

In this connection, it is also to be observed that the steel should have superior depth hardening characteristics, so that the metal will be in a uniform condition throughout, the important advantages of which are that deep cuts can be made without decrease in the unit strength, and also that irregular sections can be quenched with a minimum of warping.

Finally, as to the performance or physical properties of the article produced. The steel should have a high tensile strength and a high elastic limit, with a maximum elongation, so that, for example, accidental bending may occur and re-straightening accomplished without weakening the metal. Stated in other words, the steel should have a maximum strength with maximum capacity for cold bending. The steel should also have a very high resistance to impact and shock and to alternating stresses. These properties are essential to a commercial alloy steel, such as used in the manufacture of automobiles, and they must be obtained by the addition of alloys in amounts such as to bring the costs within allowable limits.

A steel to be commercial, therefore, must have all of the foregoing characteristics as well as certain other properties not specifically mentioned, and if it fails to substantially meet the requirements either in the

making of the steel, the forming of the steel, the physical properties of the article, or the cost, it may be dismissed as being unsatisfactory. Up to the present, it has been difficult to obtain a commercial steel which was uniformly excellent in all these respects, and it has been necessary to sacrifice to a certain extent some of the most desirable properties, in order to meet other requirements. Stated in other words, commercial steels at present in use are not well balanced, and, in addition, it has been impossible to obtain the super-excellent qualities of certain special steels without losing other properties absolutely essential to a commercial steel. To illustrate, the vanadium steel used in automobile manufacture may be considered as one of the most excellent commercial alloy steels, but, as hereinbefore pointed out, its liability to crystallization above certain narrow temperature ranges causes a large percentage of loss not only during forging, but also in the subsequent heat treatment because of the inability to maintain furnace temperatures uniform, the attempt to overcome which by means of regulating mechanism involves a very large expense without completely satisfactory results. In consequence, breakages frequently occur in service. Again, in nickel steels we find that the steel, although having non-crystallizing characteristics superior to those of vanadium steel, is very hard to machine after heat treatment. The working of such steels, therefore, involves great expense in time, labor and tools. In manganese steels, such as Hadfield steel, we find super-excellent properties such, for example, as exceedingly high tensile strength and high elastic limit, with an elongation of approximately 50%, and a relatively high reduction in area. Such steels, however, are unworkable and most difficult, if not impossible to machine. Chrome steels also fall short in some respects, particularly as to crystallization and narrow range of heat treatment.

It is the purpose of my present invention to provide a commercial alloy steel which at the same time has the super-excellent qualities of certain of the special steels, and retains all of the other characteristics necessary to bring the steel within the commercial class; these desired results being obtained at a great saving in cost and reduction in losses, as will appear.

I accomplish the foregoing by the use of molybdenum, as an added element to alloy steels, in fractional percentages ranging substantially from between 0% to 1% or a little higher. I am aware that molybdenum has been used in what is known as molybdenum high speed steel, to give such steels increased toughness and hardness and other good tool working qualities. Such steels are, of

course, impractical for commercial purposes, and their field of use strictly limited. The percentage of molybdenum used in such steel is also quite high, and the steel has not met 5 with extended use because of certain defects which develop. Relatively high percentages of molybdenum have also been used in the production of magnet steels, and in other special steels, such as armor plate, big gun 10 steel, and the like, mainly for the purpose of replacing a portion of the tungsten, and that extensive experiments have been made to observe the effect of molybdenum on iron. In so far as I am aware, however, no one has 15 made use of molybdenum in the production of commercial steels to obtain the results and advantages herein set forth; this probably because the experiments of early investigators, of the effect of molybdenum on 20 steels in the normal state led to certain conclusions indicating the presence of questionable properties from a commercial standpoint. I have found, however, that the molybdenum commercial steels, upon being 25 heat treated, apparently do not follow the laws of metallurgy, and that results are obtained opposite in character to those which would be naturally predicated from the steel in the normal state.

30 By the use of molybdenum in alloy steels, in small percentages, I find, in so far as the manufacture of the steel is concerned, that all the requirements are well met, and that in addition the molybdenum does not segregate 35 and apparently has a tendency to prevent segregation of the other ingredients alloyed. The rolling mill yield is also higher and the cost of grinding less.

Most marked results are obtained in the 40 forming of the steel. To illustrate, the forging temperature can be carried considerably higher than is ordinary without fear of destroying properties hitherto unreclaimably lost if the temperature exceeded the allowable narrow limits. In other words, the 45 forging can be done at a higher temperature without burning or over-crystallizing the steel, and this results in cutting down the forging operations because the metal is 50 more plastic, and it also eliminates the losses heretofore frequently occurring for the reason that the allowable limits of forging temperature were exceeded during the forging, because of inability to maintain uniform 55 temperature regulation, particularly where articles are being produced in large quantities. An additional saving is effected by virtue of the fact that with such wider range of forging temperature, the use of the expensive 60 regulating equipment and operators is obviated, because the furnace men can readily approximate the temperature within much less than 200°, merely by the color of the metal.

65 Again, the range of temperature for heat

treatment is greatly increased, and instead of being confined within 10° to 20° F. as is the case with present commercial alloy steels, the temperature range is increased to about 200°. Stated in other words, the 70 molybdenum prevents detrimental structural changes, such as crystallization, and secondary chemical reactions from taking place until the temperature goes several hundred degrees above the point of recalescence. This 75 is an advantage of the greatest importance, not only because of the saving effected in the cost by the elimination of furnace regulating equipment, but also because the metal will run uniformly under wide variations in temperature which means that the losses in manufacture and in service, ordinarily attributable to exceeding the narrow range of heat treatment, are reduced to a minimum, if not entirely eliminated. In other words, 80 it is possible to manufacture machine parts, for example, on a large scale and obtain uniform results notwithstanding the impossibility of maintaining uniform temperature 85 conditions.

90 Furthermore, it appears that the qualities of the steel after forging are far superior than is ordinarily found to be the case, so that it is possible, if desired, to eliminate the normalizing heat preceding the quenching 95 heat. In so far as the drawing heat is concerned, the use of the molybdenum makes it possible to draw at a much higher temperature, which effects a saving because it is much easier to regulate a furnace at high 100 temperatures than it is at low temperatures.

As to workability after heat treatment, I find that alloy steels made in accordance with my invention have excellent machining 105 characteristics, having the ease of workability of vanadium steel combined with the superior non-crystallizing characteristics of the nickel steels.

The physical properties of the steel, in contra distinction to ordinary commercial 110 alloy steels, very closely approximate the super-excellent properties of the special steels. Thus, the tensile strength and the elastic limit are greatly increased, while a maximum elongation is obtained. The cost 115 to obtain like results with the nickel and the vanadium steels, even assuming that no result detrimental to other properties would follow, would be prohibitive. The steel also has a very high resistance to impact and 120 shock and to alternating stresses without crystallization, the reduction in area is excellent, and the steel can be cold bent double or twisted a number of times, without developing flaws. It appears that by the use 125 of molybdenum in small quantities, the increase in the physical properties is obtained without a corresponding increase in the Brinell and machining hardness, which remain well below workable limits. It might 130

also be again observed, that the molybdenum materially increases the depth of hardening, so that the above properties will be found even where considerable reductions in cross-sectional areas are made during manufacture. Certain of these properties flow from the fact that the increased temperature range permits of forging, quenching and drawing at a higher temperature; and others from the direct chemical effect and the indirect chemical effect of the molybdenum.

In order to demonstrate that the temperature range of heat treatment is greatly increased without impairment of the physical properties of the steel, the following table of the properties of eight experimental test bars, of the same analysis, is given. The quenching temperatures of the bars varied through 200° F. Each bar was annealed for three hours at 1020° F. and machined down to .505" from  $\frac{3}{4}$ " hexagons. The analysis of the steel was:

|    | C.  | Mn. | Cr. | P.   | S.   | Si. | Mo. |
|----|-----|-----|-----|------|------|-----|-----|
| 25 | .24 | .65 | .46 | .021 | .031 | .17 | .44 |

The physical properties as shown by these tests were as follows:

| Bar. | Quench. | Tensile S. | E. L.   | R. A. | El. | Br. |
|------|---------|------------|---------|-------|-----|-----|
| 30   | 1500    | 144,000    | 119,000 | 47%   | 14% | 286 |
| 2    | 1520    | 144,000    | 132,000 | 52%   | 15% | 302 |
| 3    | 1540    | 148,000    | 132,000 | 49%   | 16% | 311 |
| 4    | 1560    | 147,500    | 132,000 | 50%   | 16% | 321 |
| 5    | 1580    | 148,000    | 132,000 | 51%   | 17% | 311 |
| 6    | 1600    | 145,000    | 132,000 | 49%   | 16% | 311 |
| 7    | 1650    | 149,000    | 132,000 | 51%   | 16% | 311 |
| 8    | 1700    | 151,000    | 135,000 | 50%   | 15% | 321 |

It will be observed that notwithstanding the extremely wide variation in quenching temperatures, the physical properties vary but little.

To illustrate the effect of molybdenum on chrome nickel steels, the following tables are given:

#### Analysis.

| C.  | Mn. | Cr.  | P.   | S.   | Si. | Ni. | Mo. |
|-----|-----|------|------|------|-----|-----|-----|
| .33 | .80 | 1.00 | .018 | .016 | .15 | --- | --- |

#### Properties.

|    | T. S.   | E. L.   | El.   | R. A. |
|----|---------|---------|-------|-------|
| 50 | 144,000 | 112,500 | 15.5% | 54%   |

Upon the addition of nickel 1.06% and molybdenum 0.56%, the properties were as follows:

| T. S.   | E. L.   | El. | R. A. |
|---------|---------|-----|-------|
| 180,000 | 152,000 | 16% | 53%   |

In this table all bars were quenched at 1500° F. and drawn at 1080° to 1100° F. on 1" hexagon cross sections, and test pieces machined down to .505".

It will be observed that there is a marked increase in tensile strength and elastic limit, and this with a slight increase in elongation

and with but a slight loss in the reduction in area.

The commercial value curve of nickel steels, however, begins to drop off with higher percentages of nickel, and to get the best results in commercial steels the nickel should be used in small percentages in combination with small percentages of molybdenum. The nickel should be used in quantities less than 5%, above which the steel will lose workability.

The following tables of experimental tests illustrate the effect of small percentages of molybdenum on the physical properties of chrome steels, the depth hardening characteristics of molybdenum, and the modification of the effect of section produced by the molybdenum, all bars being quenched at 1500° and drawn at 1040-1050° F. The bars were hand forged from small ingots 5" x 5" x 10" to the section indicated. They were then heat treated and standard test bars of .505" diameter were machined from the center section.

| Analysis.                                                                 | Section.          | Properties.                                            |     |
|---------------------------------------------------------------------------|-------------------|--------------------------------------------------------|-----|
| C. .286<br>Mn. .71<br>Cr. .92<br>P. .021<br>S. .025<br>Si. .28<br>Mo. .00 | 2"                | T. S. 140,000<br>E. L. 129,000<br>El. 17%<br>R. A. 58% | 90  |
|                                                                           | 1"                | T. S. 130,000<br>E. L. 112,500<br>El. 17%<br>R. A. 56% | 95  |
|                                                                           | 1 $\frac{1}{2}$ " | T. S. 130,000<br>E. L. 105,000<br>El. 16%<br>R. A. 51% | 100 |
|                                                                           | 1 $\frac{3}{4}$ " | T. S. 124,000<br>E. L. 95,000<br>El. 16%<br>R. A. 44%  | 105 |

It will be noted that the drop in tensile strength is 16,000 pounds and in elastic limit 34,000 pounds, a very clear indication that the steel has not hardened.

|                                                                | Section.          | Properties.                                                    |     |
|----------------------------------------------------------------|-------------------|----------------------------------------------------------------|-----|
| C. .294<br>Mn. .71<br>Cr. .92<br>P. .021<br>Si. .30<br>Mo. .18 | 2"                | T. S. 147,500<br>E. L. 132,500<br>El. 17.5% on 2"<br>R. A. 55% | 115 |
|                                                                | 1"                | T. S. 147,000<br>E. L. 125,000<br>El. 15%<br>R. A. 51%         | 120 |
|                                                                | 1 $\frac{1}{2}$ " | T. S. 144,000<br>E. L. 125,000<br>El. 16%<br>R. A. 52%         | 125 |
|                                                                | 1 $\frac{3}{4}$ " | T. S. 138,000<br>E. L. 110,000<br>El. 16%<br>R. A. 45%         | 130 |

Attention is called to the fact that the addition of molybdenum increases the gen-

eral properties over the first steel, and also decreases the effect of section, the drop in elastic limit from  $\frac{3}{4}$ " section to  $1\frac{1}{2}$ " section being 22,000 pounds, as compared to 34,000 5 pounds where no molybdenum is used. This indicates that the molybdenum increases the depth of hardening, as does the fact that the decrease in tensile strength is less. These effects are progressive with 10 increasing amounts of molybdenum as shown in the remaining tables of this group.

|    | Analysis.                                                                  | Section.         | Properties.                                              |
|----|----------------------------------------------------------------------------|------------------|----------------------------------------------------------|
| 15 | C. .296<br>Mn. .709<br>Cr. .94<br>P. .021<br>S. .31<br>Si. .31<br>Mo. .335 | $\frac{3}{4}$ "  | T. S. 151,000<br>E. L. 130,000<br>El. 17%<br>R. A. 58%   |
| 20 |                                                                            | 1"               | T. S. 150,000<br>E. L. 130,000<br>El. 15%<br>R. A. 55%   |
| 25 |                                                                            | $1\frac{1}{2}$ " | T. S. 142,000<br>E. L. 120,000<br>El. 15%<br>R. A. 44%   |
| 30 |                                                                            |                  |                                                          |
| 35 | C. .296<br>Mn. .71<br>Cr. .92<br>P. .021<br>S. .025<br>Si. .31<br>Mo. .515 | $\frac{3}{4}$ "  | T. S. 167,500<br>E. L. 157,500<br>El. 14.5%<br>R. A. 50% |
| 40 |                                                                            | 1"               | T. S. 174,000<br>E. L. 152,000<br>El. 14%<br>R. A. 48%   |
| 45 |                                                                            | $1\frac{1}{2}$ " | T. S. 170,000<br>E. L. 150,000<br>El. 13%<br>R. A. 37%   |
| 50 |                                                                            | $1\frac{1}{2}$ " | T. S. 170,000<br>E. L. 145,000<br>El. 11%<br>R. A. 36%   |
| 55 | C. .30<br>Mn. .72<br>Cr. .95<br>S. .025<br>P. .021<br>Si. .032<br>Mo. .77  | $\frac{3}{4}$ "  | T. S. 169,000<br>E. L. 158,000<br>El. 16%<br>R. A. 54%   |
|    |                                                                            | 1"               | T. S. 171,000<br>E. L. 145,000<br>El. 16%<br>R. A. 53%   |
|    |                                                                            | $1\frac{1}{2}$ " | T. S. 172,000<br>E. L. 150,000<br>El. 15%<br>R. A. 49%   |
|    |                                                                            | $1\frac{1}{2}$ " | T. S. 170,000<br>E. L. 150,000<br>El. 14%<br>R. A. 46%   |

From the foregoing it will be observed that, although the analysis of the various experimental steels, above considered, aside from the molybdenum content is substantially the same, the addition of the molybdenum in fractional percentages has a very

marked effect on the physical properties of the steel.

These favorable properties increase with the use of molybdenum up to 1% or a little more, and thereafter the commercial value 70 curve of the steel begins to drop off owing to the development of stiffness, brittleness and other properties, detracting from the workability of the steel, and also because the sensitiveness in the temperature of heat 75 treatment increases.

The independent effect of molybdenum on the properties of commercial steels may be emphasized by the following comparative 80 tables of tests conducted with  $\frac{3}{4}$ " hexagon bars, quenched at 1560° F. and drawn at 1020° F., the first steel being a plain unalloyed carbon steel containing .23% carbon, .81% manganese, .021 phosphorus, .025 sulfur and .25 silicon; the second steel having 85 added thereto .60% chromium and no molybdenum; the third steel having added thereto no chromium and .70% molybdenum; and the fourth steel having added thereto .60% chromium and .70% molybdenum. 90

| Tensile strength. | Elastic limit. | Elong. on 2". | Red. in area. |
|-------------------|----------------|---------------|---------------|
| 83,000            | 60,000         | 30%           | 69%           |
| 122,000           | 110,000        | 16%           | 55%           |
| 152,000           | 135,000        | 14%           | 45%           |
| 174,000           | 165,000        | 13%           | 44%           |

The results of all of the foregoing experimental tests are fully supported in later 100 actual commercial development. Thus, for example, the foregoing stock for machine parts which I prefer as giving the most satisfactory results, and the analysis of which is as follows, namely, carbon .27%, manganese .74%, chromium .96%, silicon .20%, sulfur .021%, phosphorus, .019%, and molybdenum .61%, has the following physical properties, to wit: tensile strength 170,000 pounds, elastic limit 155,000 pounds, elongation 17 $\frac{1}{2}$ % and reduction in area 61%. 110 The test piece (.505" diameter) was machined from a bar  $1\frac{1}{8}$ " square by 12" long which had been quenched at 1580° F. and drawn at 1040° F. This tensile strength together with the elongation gives an unusually high merit number to the steel. These remarkable physical properties are emphasized by the fact that, in the making of this steel, the blooming mill yield was 81%, 115 which is considerably higher than is the case in present commercial alloy steels, and the cost of preparing the ingot for rolling reduced by more than one-half, and by the further fact that the steel is readily machinable. The increase in properties is most marked when compared with those of one of the best vanadium steel at present used in automobile crank shafts, the physical properties of which substantially run as follows 120 125 130

in good practice:—tensile strength 130,000 pounds, elastic limit 115,000 pounds, elongation 19%, and reduction in area 59%. In connection with this comparison, attention is 5 called to the fact that any increase in merit number (product of elongation and ultimate tensile strength) over that of present alloy steels is remarkable.

The improvement in physical properties 10 above noted in connection with forging stock applies also to spring steels and case-hardening steels made in accordance with my invention, thus for example, in spring steels, the following physical properties may be 15 obtained, namely,

|                        |                            |
|------------------------|----------------------------|
| Tensile strength.....  | 201,000 to 270,000 pounds. |
| Elastic limit.....     | 180,000 to 225,000 pounds. |
| Elongation on 2%.....  | 7% to 15%                  |
| Reduction of area..... | 17% to 45%                 |

20 These steels also have increased resistance to dynamic stresses from which it will be readily seen that they are exceedingly desirable for springs.

Furthermore, in case hardening steels I 25 find, in steels made in accordance with my invention, the general penetration of carbon is superior, the increase in penetration of as much as 15% being obtainable which obviously improves the quality of the case formed during carbonizing.

30 In conclusion, therefore, it appears that the use of molybdenum in small percentages intensifies the effect of the other alloys, increases the most desirable physical properties, and substantially maintains greater elongation, with more excellent reduction in area percentages, and with increase of the resistance to impact and shock and to alternating stresses. Thus, I am enabled to obtain the super-excellent qualities such as 35 found in the more special steels, while at the same time the steel has all of the other properties necessary to commercial steels. The net result is a commercial steel which is far 40 superior in properties and is much cheaper both to make and to manufacture, for reasons given above. My invention is most useful in making ternary and quarternary compounds of alloy steels.

50 I do not wish to be understood as limiting myself to steels having the precise proportions of content above given, but I prefer the following proportions, as giving the best commercial results, namely:—

55 For forging stock for crank shafts, axles, connecting rods, spindles, etc., carbon from .20% to .35%; manganese from .30% to 1.25%; chromium from a fraction of a per cent. to 1.20%; silicon from .15% to .35%, and molybdenum from a fraction of a per cent. to 1%.

60 For spring steel, carbon from .38% to .55%; manganese from 40% to 1.25%; chromium from a fraction of a per cent. to 2%;

silicon from .10% to .40%; and molybdenum 65 from a fraction of a per cent. to 1%.

For case hardening steels, carbon from .06% to .18%; manganese from .20% to .75%; chromium from a fraction of a per cent. to .75%; silicon from .10% to .40%; 70 and molybdenum from a fraction of a per cent. to 1%.

It will be seen, therefore, from the foregoing that the term commercial steel covers machine parts of the class described, including 75 crank shafts, axles, connecting rods, pitmen, spindles, cams, cam shafts, gears, springs, parts to be case hardened, die blocks, hammers, parts of forging machines, particularly those undergoing heavy duty, 80 and equivalent articles; as well as certain other classes of steel of a more special nature where the molybdenum is used in substantially the proportions specified, in contradistinction to steels of a similar character 85 in which the molybdenum is embodied in much higher percentages, particularly where the molybdenum is added to bring the special steels more within the class of commercial steels.

I do not herein specifically claim the subject matter relating to spring steels specifically described and claimed in divisional application No. 184,942; the subject matter relating to case hardening steels specifically described and claimed in divisional application No. 184,940; nor the subject matter relating to chrome steels specifically described and claimed in divisional application No. 184,941; all filed August 7th, 1917. 90

I claim:

1. A commercial steel having a high merit number but readily workable, containing the usual constituents of steel and embodying molybdenum as an added element. 95

2. A commercial steel having a high merit number but readily workable, containing the usual constituents of steel and embodying molybdenum as an added element in quantities ranging from a substantial fraction of 1% to not materially more than 1%. 100

3. A commercial steel having a wide range of heat treatment, containing the usual constituents of steel and embodying molybdenum as an added element. 115

4. A commercial steel having a wide range of heat treatment, containing the usual constituents of steel and embodying molybdenum as an added element in quantities ranging from a substantial fraction of 1% to not materially more than 1%. 120

5. A steel having a tensile strength ranging approximately from 120,000 lbs. to 270,000 lbs. and an elastic limit ranging approximately from 100,000 lbs. to 225,000 lbs. 125 which contains molybdenum in addition to the usual constituents as an added element in quantities ranging from a fraction of 1%

to not materially more than 1%, the steel being characterized by workability.

6. A steel having a wide range of heat treatment and characterized by workability, substantially containing carbon from .20 to .35%; manganese from .30 to .125%; chro-

mium in relatively large traces up to 1.20%; silicon from .15 to .35%; and molybdenum in relatively large traces up to 1%.

In testimony whereof I have hereunto signed my name.

CHILD HAROLD WILLS.